

Patented Nov. 13, 1928.

1,691,764

# UNITED STATES PATENT OFFICE.

WILLIAM J. KELLY, OF AKRON, OHIO, ASSIGNOR TO THE GOODYEAR TIRE & RUBBER COMPANY, OF AKRON, OHIO, A CORPORATION OF OHIO.

## GAS-CELL FABRIC.

No Drawing.

Application filed June 23, 1925. Serial No. 39,151.

My invention relates to lighter-than-air craft and it has particular relation to gas retaining mediums employed therein.

The object of my invention is to provide 5 an inexpensive yet highly impermeable medium for retaining a buoyant fluid.

The problem of providing a suitable medium for retaining a gas has never been solved satisfactorily. This is due in part perhaps 10 to the fact that the requirements are very stringent and in part to the necessity of selecting an inexpensive material. To be satisfactory, the medium must not only be of minimum weight, but must be susceptible to 15 flexing, changes in temperature and in addition must have age-resisting qualities. Obviously, another important property which a fabric must possess is that of impermeability, especially with respect to the buoyant 20 fluid. On the other hand a medium which will retain the buoyant fluid cannot be adapted if it is not impermeable to oxygen and nitrogen. A less important consideration, but nevertheless one that should not be 25 ignored, is that of the relative solubility of the several gases. For example, gold beaters' skin, which is highly impermeable to hydrogen and helium, has a tendency to dissolve oxygen and nitrogen, and by so doing 30 dilute the buoyant fluid to such extent as to necessitate purifying it from time to time.

Heretofore many materials have been tried. Universally these embodied a suitable reinforcing medium, such as a light 35 cotton fabric, which has been impregnated or united with any one of a large number of materials, including lacquers, varnishes, rubber composition and the like. As mentioned above, gold beaters' skin has been employed. Without doubt this material is the 40 most efficient. On the other hand, it is by far the most expensive. Recently a mixture of viscose and latex has been suggested. With one exception, however, namely that 45 of gold beaters' skin, the materials lack sufficient merit to receive serious consideration.

I now have found that by using a solution of cellulose, such for example as viscose, in conjunction with a suitable reinforcing medium, it is possible to produce a material which 50 is a befitting substitute for gold beaters' skin. In practicing my invention in its preferred form, a textile material, such, for example, as to two ounce cotton fabric is coated with 55 a viscose solution containing as much as

a ten percent cellulose. Several coats are applied until the weight of the product aggregates four and a half ounces per square yard. While I prefer to apply each successive coat after the one preceding has been allowed to dry, this is not necessary and the material may be applied by a single dip.

After sufficient cellulose has been applied to give the product the required mass, the resultant film is regenerated with a weak 60 solution of sulphuric acid. During the regenerating process some hydrogen sulfide is liberated. I have found however that it is possible to prevent a permanent bubble formation in the film by first treating the material with a slightly acidified solution of sodium sulfate and subsequently passing it through the regenerating medium. The fabric is then washed free of the acid, after 65 which it is treated with a softening agent. 70 For this purpose, glycerol, which has been diluted with an equal volume of water, may be employed. It is important during the processing operations to maintain the cloth under a slight tension. In the laboratory 75 this has been effected by stretching the fabric on a frame before the initial treatment, while in production it is possible to utilize any tensioning devices for stretching the fabric, such as a tentering machine, well-known in the textile and dye industries. 80

The regenerating action is a phenomenon often met in the chemistry of colloids. The initial step is one of a setting action together with a gelatinization and dehydration and is directed toward the removal of the solvent. 90 It may be effected by utilizing any one of a large variety of materials and while I have suggested sulphuric acid, many other materials may be employed. These include 95 sodium bisulfite, formic acid, sodium-acid-sulfate, meta-bisulfite and numerous others. Furthermore, as in the manufacture of artificial silk, the cellulose may be regenerated from the viscose solution by employing a 100 progressively more concentrated coagulating medium. I have found the tensile strength and durability of the product is thereby improved.

In setting forth the details of the invention, 105 viscose has been referred to as an example of a solution of cellulose. The invention of course is not limited to this specific substance inasmuch as cuprammonium or zinc chloride solutions are available substitutes for the 110

xanthate. It will also be appreciated that the incorporation of pigments, fillers or dye materials is clearly within the scope of the invention.

- 5 The product so formed is particularly adapted to be used in rigid dirigibles. On the other hand, it is not so limited but may be used in semi-rigid and non-rigid constructions as well as ordinary balloons. In utilizing the fabric for this purpose the sheets of material may be joined by an ordinary glue splice, after which the gas cell may be varnished according to well established procedure.
- 10 15 While I have described but a single embodiment of my invention with several minor modifications thereof, it will be appreciated by anyone skilled in the art that it may be subjected to other variations without de-

parting from the spirit of the invention or 20 the scope of the claims.

What I claim is:

1. A method of rendering balloon fabric impervious to inflating gas which comprises coating the fabric with a solution of cellulose 25 xanthate containing a material inhibiting the formation of hydrogen sulphide bubbles, and re-generating the cellulose to form a uniform coating upon the fabric.

2. The method of treating balloon fabric 30 which comprises coating the fabric with a solution of cellulose xanthate containing acidified sodium sulphate and re-generating the cellulose upon the fabric.

In witness whereof, I have hereunto signed 35 my name.

WILLIAM J. KELLY.